

May 28, 1935.

V. O. ALLEN

2,002,653

ELECTRON DISCHARGE DEVICE

Filed May 24, 1930



V. O. ALLEN

INVENTOR

BY *Darby + Darby*  
ATTORNEY

## UNITED STATES PATENT OFFICE

2,002,653

## ELECTRON DISCHARGE DEVICE

Victor O. Allen, Madison, N. J., assignor, by mesne assignments, to Radio Corporation of America, a corporation of Delaware

Application May 24, 1930, Serial No. 455,297

6 Claims. (Cl. 250—27.5)

This invention relates to electron discharge devices, and with particularity to so-called indirectly heated emitters for audions or similar devices.

5 A principal object of the invention is to provide an indirectly heated cathode for audions and similar devices which has a minimum of time lag between the application of heating current and the effective emission of electrons.

10 Another object of the invention is to provide an electron emissive coating for audions or the like have a high electron emission at a comparatively low temperature.

15 Another object of the invention is to employ an electron emitting cathode for audions or the like employing caesium.

20 A feature of the invention relates to the method of applying an electron emitting coating containing caesium to a cathode or similar element such as ordinarily employed in electron discharge devices.

25 A further feature relates to an indirectly heated cathode for audions or the like which has a minimum of heat inertia.

30 Other features and advantages not specifically enumerated will be apparent after a consideration of the following detail descriptions and the appended claims.

35 While the element caesium has been known to possess electron emitting properties when subjected to heat heretofore this element has not found any commercial application in audions or the like because of the difficulty of controlling its emissivity. This is due mainly to the fact that caesium has a very low vaporizing temperature and consequently it is extremely difficult to apply the caesium and maintain it on the cathode surface. This is particularly true in so-called indirectly heated cathodes where the electron emitting material is usually sprayed onto a cylindrical and smooth surface usually known as the cathode sleeve.

40 It has been found that caesium may be employed practically as an electron emitter by combining it with a compound or mixture containing chromium. It has also been found that chromium oxide in a nascent condition has the power of adsorbing metallic caesium and prevents the caesium from leaving the cathode sleeve or the cathode filament at temperatures above 800° centigrade. At the same time the caesium is retained in the mixed condition with the chromium compound or compounds and is capable of being rendered electronically active at temperatures as low as 300°. In other words the caesium is

utilized effectively as an electron emitter between the ranges of 300° centigrade and 800° centigrade and above the latter temperature the chromium material with which the caesium is mixed prevents the volatilization or other liberation of the caesium.

5 One preferred manner of manufacturing the coating is as follows: finely divided metallic chromium is thoroughly mixed with a caesium salt such as caesium dichromate and with a suitable binder to form a liquid emulsion which is sprayed onto the surface in the usual manner. When the cathode thus coated is mounted within the audion and the latter is subjected to the usual heat treatment during the evacuating process the heat 10 causes a reaction between the chromium and the caesium salt whereby free caesium is produced and the chromium salt is changed to chromium oxide. It will of course be understood that instead of effecting this change during the evacuating process that the emulsion as sprayed on the cathode surface may be heated to produce the chemical reaction whereby caesium and chromium oxide are produced, prior to the actual mounting of the cathode within the audion or other device.

20 Referring to the drawing there is shown one preferred manner of constructing an electron emitting cathode embodying the features of the invention. The numeral 1 represents a rod of ceramic insulating material having a pair of 30 longitudinal bores 2 and 3 wherein the heater wire 4 is looped and supported. As shown, the opposite sides of the rod 1 are cut away to provide staggered notches 5 whereby the heater wire 4 is exposed at spaced intervals. Surrounding the 35 rod 1 is a sleeve 6 of metal such as nickel or the like, carrying the coating 7 containing the caesium and chromium oxide as hereinabove described. The ends of the sleeve 6 are preferably left uncoated. When the terminals of the wire 4 are 40 connected to a source of heating current the sleeve 6 is heated due to heat transmitted through the rod 1, as well as due to the heat radiated directly from the exposed portions of the wire 4. Thus 45 the rod 1 combines the advantages of having the requisite heat inertia as well as enabling the sleeve 6 to be directly heated by radiation. For a detail description of the method of forming the rod 1 reference may be had to application Serial 50 No. 441,703. As hereinabove described the coating 7 may be in the form of an emulsion containing metallic chromium mixed with a caesium salt such as caesium dichromate or the above described emulsion may be sprayed on the sleeve 6 and sub- 55

jected to heat to reduce the cæsium and to oxidize the chromium as hereinabove described.

Audions employing cathodes such as that disclosed are capable of giving the requisite high emission at temperatures as low as 300° centigrade and accidental overloads on the heater filament do not seriously volatilize or liberate the cæsium from the cathode surface.

While one specific type of heater construction is shown in the drawing, it will be understood that the invention is not limited thereto, the broad aspect of the invention residing in the method of employing and producing cæsium in a practical way to render it useful in audions or similar electron discharge devices.

Further, it will be understood that the invention is not limited to the particular materials disclosed and that various changes and modifications may be made without departing from the spirit and scope of the invention.

What is claimed is:

1. An electron emitting cathode for audions and similar devices including a member coated with cæsium-bearing material and chromium, said cæsium bearing material being capable of reduction by chromium to produce chromium oxide.

2. An electron emitting cathode for audions and similar devices comprising a member having a coating of metallic cæsium and chromium oxide.

3. A mixture for preparing an electron emissive member comprising metallic chromium and cæsium dichromate.

4. In an electron emitter for vacuum tubes the combination of a rod of insulation having a longitudinal bore therethrough and a plurality of undercut notches, exposing said bore at spaced intervals, a heater wire threaded through said bore, a metallic sleeve surrounding said rod and an electron emissive coating containing cæsium and a material containing chromium on the exterior surface of said sleeve.

5. The step in the method of manufacturing an emissive cathode for electron discharge devices which comprises mixing cæsium di-chromate with comminuted chromium, applying the resultant mixture to a cathode support, and subjecting the whole to heat treatment to reduce the cæsium compound to the metal cæsium.

6. An emitting cathode for audions or similar devices comprising a member having a coating of cæsium compound which is electronically active in the neighborhood of 300° C. and which is capable of reduction by chromium to produce chromium oxide and provided with metallic chromium for preventing loss of the emitting material at higher temperatures.

VICTOR O. ALLEN.

30